

2 Sheets--Sheet 1.

Z. S. DURFEE.

Improvement in Casting Ingots.

No. 122,310.

Patented Jan. 2, 1872.



Fig. 1.

John C. Myman  
John L. Swift  
John S. Durfee

2 Sheets--Sheet 2.

Z. S. DURFEE.

Improvement in Casting Ingots.

No. 122,310.

Patented Jan. 2, 1872.

Fig. 3.



Fig. 5.



Fig. 4.



Fig. 2.



John C. O'Byrne  
Witness - Z. S. Durfee Inventor.

John C. O'Byrne  
Witness - Z. S. Durfee Inventor.

## UNITED STATES PATENT OFFICE.

ZOHETH S. DURFEE, OF NEW YORK, N. Y.

## IMPROVEMENT IN CASTING INGOTS.

Specification forming part of Letters Patent No. 122,310, dated January 2, 1872.

I, ZOHETH S. DURFEE, of the city, county, and State of New York, have invented a new and Improved Mode of Making Long Shafts of Steel, and of Constructing and Arranging Ingot-Molds for Casting Ingots therefor, of which the following is a specification:

My improvement consists in casting the ingots for long shafts in a bent form and then straightening them; and my purpose is, first, to avoid having the melted metal for the ingots fall through a very great height, and to be able to make a long shaft without having to draw it from an ingot of large diameter.

In the drawing, Figure 1 shows my molds partly in a vertical position and partly in elevation; Fig. 2, a transverse section of the sprue molds and base through the connected molds; Fig. 3, a plan of the base plate; and Figs. 4 and 5, cross-sections of the molds.

*a* is the sprue mold; *b b*, the connected molds; *c*, the base; *d*, the base plug or center plate for taking the stream of metal; *e e*, the snugs or ears whereby the connected molds are held together; *f f*, the connecting bolts; *h h*, the eyes for handling the molds; *g*, the runner from the sprue to the connecting mold, which is here shown without lining, but may be made larger, and belined with refractory material, if desired. The sprue molds and the connected molds are separated somewhat by a projection, *i*, on the sprue mold, partly to allow room for the connecting bolt, and partly to allow a play of air

between them and lessen the liability of their becoming too highly heated by the flowing metal. The operation of the molds will be clearly understood from the drawing.

I make the bent ingot sufficiently large at the angle to allow cutting away all the sprue and a part of the metal adjacent thereto, so as to insure sound metal throughout the length of the ingot.

In making long shafts on this plan I prefer to make the ingots of a section only so much larger than the shaft required as will allow a proper condensation of the metal without much elongation.

This angular arrangement of ingots may be effected without a sprue mold, the two angular ingot-molds being set on a base, as shown, and filled by pouring the metal into the upper end of either one of them.

What I claim as my invention is—

1. Making long shafts or other pieces of steel by first casting ingots in a bent form and then straightening and drawing and condensing said ingots, substantially as and for the purposes specified.

2. The arrangement and construction of ingot-molds for casting bent ingots, substantially as shown in the drawing herewith.

ZOHETH S. DURFEE.

Witnesses:

EMIL FLEUSNER,  
CHI. H. LADDING.

(33)